

# UNITED STATES PATENT OFFICE.

AUBREY E. MEYER, OF NEW YORK, N. Y.

## TEXTILE YARN AND METHOD OF MAKING THE SAME.

1,295,821.

Specification of Letters Patent. Patented Feb. 25, 1919.

No Drawing.

Application filed April 7, 1917. Serial No. 160,494.

To all whom it may concern:

Be it known that I, AUBREY E. MEYER, a citizen of the United States, and a resident of the borough of Manhattan, county and State of New York, have invented certain new and useful Improvements in Textile Yarn and Methods of Making Same, of which the following is a specification.

My invention relates to textile yarn and method of making same. One of the objects of the invention is to provide a fibrous "yarn" or so-called "thread" of the character used in textile fabric of the interlaced strand type, having sufficient strength for such use, and having its fibers lying more parallel than has heretofore been accomplished, whereby the appearance and quality of certain kinds of such fabric are greatly improved. By "more parallel" I mean lying side by side in a more longitudinal direction. By a fabric of the interlaced strand type I mean one whose strands are interlaced one with the other, such for example as woven fabric, or one whose strand is interlaced on itself as for example knitted fabric, etc.

Another object of the invention is to provide a novel and efficient method of making such yarn.

My invention comprises, in its broader aspect, the replacing of a substantial amount, or all, of the otherwise necessary twist in such fibrous yarn of any particular specie, by a suitable adhesive, and this is accomplished according to my invention by twisting such yarn having a suitable adhesive thereon or therein. The invention does not contemplate the application of an adhesive to yarn for the purpose of further strengthening twisted yarn beyond the strength that such yarn would have if given the usual necessary twist to enable it to be handled and used in making fabrics of the above type, for the strengthening of thread and other strands by the application of an adhesive such as wax is well known, as well as is the coating of strands with an adhesive to protect the strand from abrasion, or to render it waterproof in fabric. But the invention provides for a more parallel arrangement of the fibers themselves of such yarn or "thread" for various purposes; and to accomplish this, the strengthening factor—"twist"—is partially or substantially wholly replaced by the other strengthening factor—adhesive. The decrease in twist,—i. e., a more parallel arrangement of the

fibers in the yarn, is very desirable for many purposes, among which the following may be mentioned. It gives to the yarn a better filling quality or greater fullness or loftiness for the same weight of yarn, and in most instances a higher luster. A fabric made from yarn or threads according to my invention, can be more easily waterproofed after being fabricated. It will also "take" any coating more readily and probably more rigidly, such as coatings to manufacture imitation leather or glazed cloths, etc. It can also, especially when knitted, be more easily "combed open" "teazled" so as to give the product a napped, woolly or hairy or fur-like appearance. It will thus be seen that my invention does not deal with the protection or additional strengthening of yarn having the usual or heretofore necessary twist, but it deals rather with the elimination of a substantial amount of the heretofore necessary twist, or substantially all or all of the twist, with a view of acquiring greater luster and loftiness in fabrics made therefrom and also other resulting properties.

Yarn made according to my invention may or may not be stronger than it would be with substantially more twist and no adhesive, and the invention is unconcerned with the relative strength of the two, so long as the untwisted and gummed yarn of the invention has sufficient strength to be handled in its manufacture and used in making fabric of the interlaced strand type.

In referring herein to yarn having substantially less twist than heretofore obtainable, and in other such expressions of comparison, I intend to compare or contrast a yarn that is otherwise the same—yarn made of fibers of a certain specie, such for example as cotton or wool, and of a certain or given graded length, for obviously a yarn of a particular size made, for example, from cotton with fibers  $1\frac{1}{2}$  inches long, such as sea island cotton, is not the same specie as the same size yarn made from cotton of a shorter staple, say one inch long. And likewise, yarn made from wool the "fibers" of which are say for example of a grade  $1\frac{1}{2}$  inches long, is not the same specie as a yarn made from cotton whose fibers are  $1\frac{1}{2}$  inches long; so that the only way in which relative amounts of twist in yarn can be compared or considered, is to compare the effect of the same yarn i. e., one of the same specie and length of fiber with more or less twist.

I have observed, other things being equal, that the less twist a yarn has—*i. e.*, the more parallel its fibers, the greater is the gloss or luster of the fabric woven therefrom; 5 and the greater is the fullness of the yarn. For example, if a yarn of a given specie has say fifteen twists to the inch and is of a certain “size” (the size being determined by the length of yarn spun from a given weight 10 of fiber), when the yarn is partially untwisted its fibers are not held together so closely and the “bulk” of the yarn increases, and this continues as the untwisting of the 15 yarn is continued, until the fibers lie substantially parallel; so that if a piece of cloth is woven from the fully twisted yarn, and a piece woven from the partly twisted yarn, a comparison of the two pieces of cloth will show that the piece woven from the fully 20 twisted yarn is more wiry, thinner and harder than the other, and has larger interstices or air spaces between its interlocked threads—*i. e.*, lacks homogeneity; whereas, the piece woven from the partially untwisted 25 yarn is softer, thicker and more uniform—*i. e.*, has less air space area, or, in other words, is a more lofty piece of goods, and in addition, has more luster, provided the yarn is of a specie having luster. This last feature 30 is of special importance in silk fabrics and in certain woolen fabrics, notably mohair and similar luster fabrics.

In view of the fact that the less twist that is given a yarn in spinning it the greater is 35 the length of yarn that can be spun from a given amount of stock, and the greater is the amount of yarn that can be produced in a given time it has been the aim of spinners, except in manufacturing yarn to be used in 40 weaving wiry, porous, or certain ribbed goods, to manufacture yarn of any specie with as little twist as has been found requisite to the strength of the yarn for its being successfully handled commercially in winding 45 it upon and unwinding it from bobbins and for subsequent use in weaving, etc. Long or high-grade fibers obviously require less twist per inch to hold them together than is required by short fibers, and the minimum 50 amount of twist required for yarn of a given specie has been rather definitely determined by usage and practice, however, varying in practice over a very small percentage range.

By my invention I am enabled to substantially 55 reduce the otherwise necessary amount of twist in fibrous yarn of any particular specie while retaining the necessary workable strength of the yarn; or to form yarn with the necessary workable strength and 60 with substantially no twist, which is sufficiently smooth, homogeneous and flexible to permit its being woven with the same apparatus and in the same manner as ordinary yarn.

65 The invention will be more readily un-

derstood by first describing the preferred method of forming yarn embodying my invention, which is as follows:

I take yarn after it has been spun in the usual manner, from sliver, roving, etc., and 70 wound upon suitable bobbins or cops, and having the necessary twist for being so handled and for permitting it to be gummed, and I then gum it in any suitable manner; as for example by passing it over gummed 75 rolls or through a suitable basin containing the adhesive, and after it has been gummed I brush it, if desired, as it leaves the rolls or basin, and then dry it as it leaves the brushes, if used, so that the gum will bind the fibers 80 together. I then take out a substantial amount or substantially all of the twist, as may be desired in the particular case; depending upon the gum wholly or in part to hold the fibers together so as to give the yarn 85 its necessary strength for use in forming said fabrics of the interlaced strand type. The twist may be taken out in any way desired, as by placing the cop in a twisting frame and rotating it in a direction to untwist the 90 yarn, as is practised in the art with un-gummed yarn, but I do not wish to limit myself to any particular manner of taking out the twist. Or, instead of taking a spun 95 yarn that has already been copped, and gumming, untwisting and recopping it, I may gum it during the spinning operation—*i. e.*, after twist has been put in it by the spinning of the yarn and before it is wound upon the cop or pirn; after which the twist 100 may be taken out as described.

Yarn thus formed may then be used for weaving or knitting fabric or otherwise making fabric of the interlocked strand type, and after the fabric has been woven or knitted in any well-known manner, I then dissolve out the gum or adhesive from the fabric. Any suitable adhesive may be used that can be readily dissolved from the fabric, such for example as glue, gelatin, 110 starch, etc. The interlocking or interlacing of the yarn or threads of the fabric one on or with the other, gives the fabric the necessary strength after the adhesive has been dissolved from the yarn or threads. 115

It will be observed that yarn made according to my invention from long high-grade fibers, has ample strength and may have its fibers lying more parallel than has heretofore been possible in any fibrous yarns of 120 sufficient strength to be wound upon or unwound from bobbins when spun, or capable of being woven into fabric; and that when it is desired, the fibers of such yarn may have substantially no twist, thus obtaining the 12 maximum benefit of the invention as regards both luster and fullness of the fabric. But it will also be apparent that yarn made according to my invention from shorter and inferior fibers of a given specie, likewise has 13

ample strength and will have its fibers lying substantially more parallel than would have been otherwise possible in the same yarn; and that this yarn with inferior fibers can 5 be made to have its fibers lying even more parallel than has been heretofore practical with the highest grade fibrous yarns, thereby making it possible to obtain with a cheaper grade of yarn having comparatively short 10 fibers, a woven fabric of a high luster and better filled than has been heretofore obtained with a high grade yarn with much longer fibers. In addition to these advantages, the length of the yarn obtainable from 15 a given amount of stock is increased proportional to the amount of twist dispensed with.

As showing the necessity of twist in yarns heretofore and the narrow range of reductions heretofore permissible from the minimum 20 amount of twist used in practice in yarns of different species,—or, in other words, as showing the well-defined minimum limits in twists, it will be helpful to consider one or two species by way of example. But 25 I will first state by way of explanation as to requisite strength of yarns, that in the manufacture of a yarn (used for weft strands) ready for weaving, the greatest strength required of the yarn is in the unwinding of it from bobbins after it is spun; while the use of the yarn as a weft strand in weaving requires less strength. Whereas, the use of the yarn as a warp strand in weaving in some species of yarn requires 30 sizing to protect it from the chafing action of the skidding operation of the shuttle, etc.; and the yarn, to stand the operation of sizing as it is practised, requires even greater strength than is required in unwinding the 35 yarn; and hence yarn that is to be sized for use as a warp strand, requires more twist than is necessary to unwind the yarn from a bobbin or cop.

With this understanding of the requirements of strength in a yarn for the different 40 operations, if we consider a high-grade 20-1 cotton yarn made of sea island cotton, where the staple or fiber is  $1\frac{1}{8}$  inches long, it has been observed from practice that "7 45 turns" (which means 7 turns or twists per inch) is sufficient for the use of the yarn as a weft strand in weaving, provided the yarn is spun directly onto the cop or pirn that is to be used in the shuttle, but yarn 50 with 7 turns is not strong enough to be recopied or wound from one cop or bobbin onto another; and the same yarn with 6 turns can be spun but cannot be unwound from a cop or pirn when in the loom, without 55 breaking. It is thus seen that in this instance a reduction of one twist in seven is the difference between success and failure in the use of this yarn; while the same yarn, to have sufficient strength to withstand the 60 operations necessary for it to pass through 65

to prepare it as a warp strand for weaving, such as spooling, warping and slashing, will require from 14 to 15 turns.

In the case of cotton yarn of another species, for example a 20-1 cotton yarn made from a staple  $1\frac{1}{4}$  inches long, 9 turns per inch is sufficient in practice for unwinding the yarn from bobbins and utilizing it as a weft strand in weaving, while 8 turns is insufficient. It will thus be seen that with this species, one turn in nine is the difference between success and failure as regards weaving.

It will thus be seen that by my invention a fabric can be obtained from yarn of a given species that is more valuable and desirable for many purposes than could have been made from the same yarn without my invention.

By the term "gummed" or "gumming" as used in the appended claims, I do not wish to be understood as limiting myself to a gum in the strictest sense of the word as distinguished from other forms of adhesive, but wish to be understood as including the use of any suitable form of adhesive, the important thing being that a suitable adhesive is present in the yarn when the same is un-twisted so as to bind the fibers together. Where in the specification and claims I use the word "untwisted", referring to yarn, I use it in its ordinary meaning, namely, as defining a yarn having a partially or wholly removed previous twist, and do not mean by such word to refer to yarn which has either not been twisted at all or has been slightly twisted and remains in that condition. And by the term "recopping" I wish to be understood as meaning the coiling or winding or re-coiling or re-winding of the yarn upon any suitable form of support or in any suitable manner in such compact form as to enable subsequent handling, shipping or use of the same.

While I have described my invention in detail according to the preferred manner of carrying out my process, it will be obvious to those skilled in the art, after understanding my invention, that changes and modifications may be made therein without departing from the spirit or scope of my invention, and I aim in the appended claims to cover all such changes and modifications.

Having thus described my invention, what I claim as new and desire to secure by Letters Patent, is:—

1. The method of forming fibrous yarn of the character used in the manufacture of textile fabric of the interlaced strand type, which comprises applying an adhesive to a twisted yarn and then sufficiently untwisting it to obtain a yarn with the desired lack of twist and requisite strength.

2. The method of forming fibrous yarn of the character used in the manufacture of

textile fabric of the interlaced strand type, which comprises twisting and gumming the fibers of the yarn and then untwisting them.

3. The method of forming fibrous yarn of 5 the character used in the manufacture of textile fabric of the interlaced strand type, which comprises taking twist out of a gummed twisted yarn.

4. The method of forming fibrous yarn of 10 the character used in the manufacture of textile fabric of the interlaced strand type, which comprises taking the twist out of a gummed, twisted and dried yarn.

5. The method of forming fibrous yarn 15 of the character used in the manufacture of textile fabric of the interlaced strand type, which comprises forming the yarn with the requisite twist for strength, applying an adhesive, and then untwisting the yarn to obtain 20 a yarn with the desired lack of twist and requisite strength.

6. The method of forming fibrous yarn of 25 the character used in the manufacture of textile fabric of the interlaced strand type, which comprises applying an adhesive to a yarn having twist, untwisting it, and recop-

ping it after it has dried sufficiently to permit recopping without the coils sticking together.

7. The method of forming fibrous yarn of 30 the character used in the manufacture of textile fabric of the interlaced strand type, which comprises applying an adhesive to a yarn having twist, allowing the adhesive to dry, and then taking the twist out and recopping. 35

8. The method of forming fibrous yarn of the character used in the manufacture of textile fabric of the interlaced strand type, which comprises applying an adhesive to a 40 yarn having twist, allowing it to dry sufficiently to bind the fibers to give the yarn the necessary strength for untwisting it, and then untwisting the yarn.

9. As a product of manufacture, a gummed 45 untwisted fibrous textile yarn of the character used in the manufacture of textile fabrics of the interlaced strand type.

In testimony whereof, I have signed my name to this specification.

AUBREY E. MEYER.